

2,722,516

**GREASE COMPOSITIONS CONTAINING  
AN ANTRUST**

Robert L. Merker, Washington, D. C.

No Drawing. Application March 27, 1951,  
Serial No. 217,900

9 Claims. (Cl. 252—40)

(Granted under Title 35, U. S. Code (1952), sec. 266)

This invention relates to improved greases embodying an antirusting agent as part of the composition. The greases to which the invention relates are those in which a metal soap is used in thickening the lubricating fluid. The invention also relates to metal soaps containing an antirusting agent.

Rusting of steel parts is often encountered where greases are used as the lubricant. Moisture deposited on the grease is transferred to the lubricated steel surface by the conjoint action of the soap and the moving part. The soap acts in the role of emulsifier for the water which is brought into emulsion with the lubricating fluid and subsequently moved to the steel surface through the continual working of the grease by the moving part. Corrosion by rusting also may occur in the case of iron-bearing parts packed with grease for storage or shipment where the grease film, either initially or through accidental rubbing off, is quite thin. In such case, moisture, such as rain, or condensate from the atmosphere, can penetrate through the thin grease film to cause rusting of the iron bearing surface.

I have found that protection against rusting can be incorporated in greases when there is added to the grease a water-soluble salt of certain carboxylic acids herein-after more fully identified.

According to the present invention, greases having antirust properties can be obtained by providing in the grease a water-soluble salt of an alkyl monocarboxylic acid of 6 to 10 carbon atoms or of an alkylene dicarboxylic acid of 7 to 20 carbon atoms. The hydrocarbon group of the acids may be branched or unbranched. The water-soluble salt is the neutral salt of the dicarboxylic acids. Suitable carboxylic acids for forming the acid portion of the salts are, for example, hexanoic, heptanoic, octanoic, 2-nonanoic and decanoic acid of the monocarboxylic series and pimelic, suberic, tetramethyl succinic, azelaic, heptyl malonic, butyl adipic, sebacic, dodecanedioic, tetradecanedioic and hexadecanedioic acid of the dicarboxylic series. A preferred group of acids for the salts are the dicarboxylic acids having from 8 to 10 carbon atoms, e. g., suberic, azelaic and sebacic acids. The salt-forming group of the water-soluble salts may be taken, for example, from the alkali metals, the alkaline earth metals, ammonium, and water-soluble amines. The sodium salts constitute a preferred group of the water-soluble salts of the afore-defined classes of carboxylic acids for preparing the improved greases of the invention.

These antirust salts are not soluble in the greases or the soap used for thickening the same, and accordingly, are dispersed therein by some suitable means, as, for example, by milling the grease with the salt in finely divided form on a three roll mill. The amount of the salt added may be varied somewhat depending upon the degree of rust prevention desired and the activity of the particular salt selected. In general it will be found that between about .05% and about 0.2% by weight of the salt on the grease will be found sufficient to give complete protection against rusting of iron-bearing surfaces lubricated

with the greases. Instead of adding the salt to the grease, it may be incorporated in the soap which is then used for thickening of the lubricating fluid to form the grease.

The water-soluble salts function in the grease as anti-rusts by dissolving in the water at the metal surface to form a salt solution from which the salt is preferentially adsorbed to the metal surface to form a layer thereon constituting a barrier between the metal and the water.

The invention is further illustrated by the results appearing in the table below and obtained from comparative corrosion tests in which a series of water-soluble salts were employed including certain of the above defined carboxylic acid salts. The tests were performed by immersion of a clean, cold rolled steel strip (1½" x ¾") in a water (tap) solution of the salt for the stated periods of time at a temperature of 80° C. The pH of all the salt solutions was approximately 8.

Table

| 20 | Salt             | Percent Weight of Salt | Appearance of Metal Specimen After— |             |           |             |
|----|------------------|------------------------|-------------------------------------|-------------|-----------|-------------|
|    |                  |                        | 3 hours                             | 24 hours    | 100 hours | 1,000 hours |
| 25 | Sod. benzoate    | 0.2                    | bad rust                            | —           | —         | —           |
|    | Sod. phenolate   | 0.2                    | do                                  | —           | —         | —           |
|    | Sod. acetate     | 0.2                    | do                                  | —           | —         | —           |
|    | Sod. laurate     | 0.2                    | slight rust                         | much rust   | —         | —           |
|    | Sod. stearate    | 0.2                    | very slight rust                    | slight rust | —         | —           |
| 30 | Sod. hexanoate   | 0.2                    | no rust                             | no rust     | no rust   | no rust     |
|    | Sod. heptanoate  | 0.2                    | do                                  | do          | do        | Do.         |
|    | Sod. 2-nonanoate | 0.2                    | do                                  | do          | do        | Do.         |
|    | Sod. oxalate     | 0.2                    | bad rust                            | —           | —         | —           |
|    | Sod. malonate    | 0.2                    | do                                  | —           | —         | —           |
|    | Sod. succinate   | 0.2                    | do                                  | —           | —         | —           |
|    | Sod. adipate     | 0.2                    | do                                  | —           | —         | —           |
| 35 | Sod. suberate    | 0.2                    | no rust                             | no rust     | no rust   | no rust     |
|    | Sod. azelate     | 0.2                    | do                                  | do          | do        | Do.         |
|    | Sod. sebacate    | 0.2                    | do                                  | do          | do        | Do.         |
|    | Borax            | 0.2                    | slight rust                         | much rust   | —         | —           |

N. B. Test discontinued in runs where positive evidence of rusting. The sodium salt of the indicated dicarboxylic acid is the neutral salt in each case.

Under the same conditions and using as inhibitor, respectively, potassium, lithium, calcium, barium, strontium, magnesium, methyl and isopropyl amine azelates (neutral salts) in a concentration of slightly less than 0.2% by weight, no rusting of the steel strip was observed even after a period of 100 hours immersion in the aqueous solution of the salt.

The rust inhibitors of the present invention can be used in a wide variety of greases both from the standpoint of the lubricating fluid and the soap used as thickener. The most common greases are those in which a petroleum oil is thickened with sodium or calcium stearate. However, the inhibitors may not only be used effectively in these common greases but likewise in greases in which the lubricating fluid is of synthetic origin, such as the diesters (alkyl esters of alkylene dicarboxylic acids), silicones, and polyalkylene oxide fluids, e. g., polyisopropylene oxide, which have been stoppered at both ends with an alkyl group, e. g., butyl, and the thickener is a metal soap of other, limitedly water-soluble higher fatty acids, e. g., lithium palmitate, aluminum stearate, etc.

Since various changes may be made in the practice of the invention described herein without departing from the spirit or scope thereof, it is to be understood that the foregoing description is intended by way of illustration and not in limitation of the invention.

The invention described herein may be manufactured and used by or for the Government of the United States of America for governmental purposes without the payment of any royalties thereon or therefor.

What is claimed is:

1. An improved lubricant grease comprising a base lubricating fluid thickened with a metal soap and containing a small, rust-inhibiting proportion of a water-soluble neutral salt of an alkylene dicarboxylic acid of 8 to 10 carbon atoms in which the carboxylic acid groups are linked to the opposite terminals of an alkylene chain of from 6 to 8 carbon atoms.

2. An improved lubricant grease comprising a base lubricating fluid thickened with a metal soap and containing a small, rust-inhibiting proportion of a neutral alkali metal salt of an alkylene dicarboxylic acid of 8 to 10 carbon atoms in which the carboxylic acid groups are linked to the opposite terminals of an alkylene chain of from 6 to 8 carbon atoms.

3. An improved lubricant grease comprising a base lubricating fluid thickened with a metal soap and containing a small, rust-inhibiting proportion of the neutral sodium salt of an alkylene dicarboxylic acid of 8 to 10 carbon atoms in which the carboxylic acid groups are linked to the opposite terminals of an alkylene chain of from 6 to 8 carbon atoms.

4. An improved lubricant grease comprising petroleum lubricating oil thickened with an alkali metal soap and containing a small, rust-inhibiting proportion of the neutral sodium salt of an alkylene dicarboxylic acid of 8 to 10 carbon atoms in which the carboxylic acid groups are linked to the opposite terminals of an alkylene chain of from 6 to 8 carbon atoms.

5. An improved lubricant grease comprising petroleum lubricating oil thickened with an alkaline earth metal soap and containing a small, rust-inhibiting proportion of the neutral sodium salt of an alkylene dicarboxylic acid of 8 to 10 carbon atoms in which the carboxylic acid groups are linked to the opposite terminals of an alkylene chain of from 6 to 8 carbon atoms.

5

6. An improved lubricant grease comprising a petroleum lubricating oil thickened with an alkali metal soap and containing a small, rust-inhibiting proportion of sodium suberate.

7. An improved lubricant grease comprising a petroleum lubricating oil thickened with an alkali metal soap and containing a small, rust-inhibiting proportion of sodium azelate.

8. An improved lubricant grease comprising a petroleum lubricating oil thickened with an alkali metal soap and containing a small, rust-inhibiting proportion of sodium sebacate.

9. An improved lubricant grease comprising petroleum lubricating oil thickened with a metal soap and containing a small, rust-inhibiting proportion of a water-soluble neutral salt of an alkylene dicarboxylic acid of 8 to 10 carbon atoms in which the carboxylic acid groups are linked to the opposite terminals of an alkylene chain of from 6 to 8 carbon atoms.

20

15

20

25

25

30

30

35

References Cited in the file of this patent

UNITED STATES PATENTS

|           |                   |               |
|-----------|-------------------|---------------|
| 2,363,514 | Farrington et al. | Nov. 28, 1944 |
| 2,363,515 | Farrington et al. | Nov. 28, 1944 |
| 2,363,516 | Farrington et al. | Nov. 28, 1944 |
| 2,368,602 | Weiss             | Jan. 30, 1945 |
| 2,426,496 | Farley            | Aug. 26, 1947 |
| 2,457,586 | McGrogan          | Dec. 28, 1948 |
| 2,481,372 | Fuchs             | Sept. 6, 1949 |
| 2,487,080 | Swenson           | Nov. 8, 1949  |
| 2,495,651 | Butcosk           | Jan. 24, 1950 |
| 2,528,373 | Knowles et al.    | Oct. 31, 1950 |
| 2,539,503 | Zisman et al.     | Jan. 30, 1951 |
| 2,583,607 | Sirianni          | Jan. 29, 1952 |